

## UNITED STATES PATENT OFFICE

2,488,662

## METAL ORGANO-PHOSPHATES

Bruce B. Farrington, James O. Clayton, and John T. Rutherford, Berkeley, Calif., assignors to California Research Corporation, San Francisco, Calif., a corporation of Delaware

No Drawing. Application June 25, 1946.  
Serial No. 679,262.

7 Claims. (Cl. 260—429)

1

This invention relates to high molecular weight, water-insoluble, mineral oil-soluble zinc and cadmium salts of acid esters of phosphoric acid.

The polyvalent metal salts of acid esters of phosphoric acid have value as improvement agents for mineral lubricating oils. Thus, they are effective, when used alone, to increase the resistance of such oils to oxidation and they have particular value, when used in combination with a polyvalent metal salt of an alkyl phenol, to inhibit corrosion of alloy bearings such as copper-lead bearings. See, for example, Farrington et al., United States Patent No. 2,228,659 and Neely et al., United States Patent No. 2,228,671.

For convenience, these polyvalent metal salts of acid esters of phosphoric acid will be frequently referred to as polyvalent metal phosphates.

Certain of these polyvalent metal phosphates, such as the calcium and barium salts, are water-soluble to a sufficient extent, or their solubilities in mineral lubricating oils are sufficiently low that difficulty is encountered in practice. Thus, it is a common practice to disperse the polyvalent metal phosphate in oil in relatively large amount, of the order of 50% on the weight of oil-phosphate solution, to produce a concentrate or stock solution. This concentrate is stored and shipped, to be blended with more oil to produce a finished product containing about 0.25 to 2.0% of phosphate. The aforesaid calcium and barium phosphates are difficult to blend homogeneously into such concentrates; and even finished oils containing lesser amounts are prone to form emulsions on agitation with water, or they may fail to pass stringent acceptance tests which include centrifuging at high speed.

Certain other polyvalent metal phosphates, such as the aluminum phosphates, although more oil-soluble and less water-soluble, cause some difficulty owing to wear of working parts of internal combustion engines, such as cylinder and piston walls and piston rings.

The above-mentioned oil-water solubility difficulties can be solved by employing phosphoric esters of sufficiently high molecular weight alcohols or phenols, but to obviate these difficulties fully it is necessary, by this means, to use esterifying radicals of excessively high molecular weight. These excessively high molecular weight radicals are more expensive than the more common radicals of lower molecular weight, containing 5 to 20 carbon atoms. Also, the esterifying radical functions primarily as an oil-solubilizing agent and the effective inhibiting action of the phosphate is imparted by the inorganic (metal-oxygen-phosphorus) group. To the extent, there-

2

fore, that hydrocarbon radicals of very high molecular weight are employed, the chemical activity of the phosphate is reduced. That is, a phosphate can be rendered more oil-soluble by employing hydrocarbon radicals of very high molecular weight, but this necessitates use of more phosphate to obtain the desired effect. Hence, the means defeats the object to a considerable extent; the phosphate is more oil-soluble but more of it is required.

It is an object of the present invention to provide a class of polyvalent metal salts of acid esters of phosphoric acid which are more oil-soluble and less water-soluble than the alkaline earth metal salts of these esters.

It is a further object of the invention to provide a class of polyvalent metal salts of acid esters of phosphoric acid which are more oil-soluble, less water-soluble than the alkaline earth metal salts of these esters and which do not cause as much wear (when used in mineral lubricating oils in engine lubrication) as aluminum salts of these esters.

It is a particular object of the invention to provide a class of polyvalent metal salts of acid esters of phosphoric acid which are oil-soluble and water-insoluble, which are characterized by low wear (in the sense above indicated) and which contain as the esterifying substituents, radicals containing 5 to 20 carbon atoms.

These and other objects of the invention will be apparent from the ensuing description and the appended claims.

We have discovered that the zinc and cadmium salts of acid esters of phosphoric acid are superior in that they are characterized by low water-solubility and high oil-solubility. Moreover, they do not cause excessive wear of working parts of machinery lubricated by mineral oils containing them.

The salts of the invention are of two types, derived from the mono-esters and the di-esters:



Salts of the mono-esters may be normal salts ( $\text{MR}_1\text{PO}_4$ ) or acid salts ( $\text{R}_1\text{HPO}_4$ — $\text{M}-\text{R}_1\text{HPO}_4$ ). In the above formulae,  $\text{R}_1$  and  $\text{R}_2$  are hydrocarbon radicals (which may be substituted, however, by non-hydrocarbon substituents) and  $\text{M}$  is zinc or cadmium. Basic salts may also be formed from

either the mono- or the di-esters. Normal salts of the types



are preferred, and of these the salts of the di-esters are preferred as being more oil-soluble. The radicals  $R_1$  and  $R_2$  contain each not less than 5 carbon atoms, preferably not less than 10 carbon atoms, and preferably not more than 20 carbon atoms. These radicals may be alkyl (e. g., amyl, hexyl, octyl, decyl, lauryl, tetradecyl, cetyl and eicosyl), alkylene (e. g., octenyl, hexadecenyl), cycloaliphatic (e. g., naphtenyl, cyclohexyl and methylcyclohexyl), aryl (e. g., phenyl), alkaryl (e. g., methylphenyl and cetyl phenyl), or aralkyl (e. g., benzyl, phenylstearyl and cetylbenzyl) radicals. Saturated aliphatic and cycloaliphatic radicals and aryl radicals substituted by one or more saturated aliphatic or cycloaliphatic radicals are preferred.

Mixed radicals, e. g., alkyl-cycloaliphatic and alkylalkaryl, may be used. Likewise, mixed salts of mono- and di-esters may be used, e. g., mixed zinc salts of mono-cetyl phosphoric acid and dicetyl phosphoric acid.

The parent esters of the salts of the invention can be prepared by methods well known in the art. Certain of the parent esters, e. g., mono- and dicetyl phosphates and mono- and dicholesteryl phosphates are described in the literature. Exemplary methods of preparation are provided by the specific examples below and by Plimmer and Burch, *Journal of the Chemical Society*, 1929, pages 279-291.

The zinc and cadmium salts can be readily prepared from the parent esters, or from alkali metal salts of the same, by methods well known in the art, as exemplified by the specific examples and by Plimmer and Burch, *op. cit.*

Examples of salts of the invention are: normal zinc and cadmium mono-amyl phosphates, normal zinc and cadmium mono-octyl phosphates, normal zinc and cadmium mono-lauryl phosphates, normal zinc and cadmium mono-eicosyl phosphates, normal zinc and cadmium mono-methylcyclohexyl phosphates, normal zinc and cadmium mono-benzyl phosphates and normal zinc and cadmium mono-cetylphenyl phosphates; also, the corresponding normal zinc and cadmium di-amyl, di-octyl, di-lauryl, di-eicosyl, di-methylcyclohexyl, di-benzyl and dicetylphenyl phosphates.

The following specific examples will serve further to illustrate the preparation and properties of the salts of the invention.

#### EXAMPLE 1

##### *Mono- and di-cetyl phosphoric acids and zinc and cadmium salts of the same*

A mixture of mono- and dicetyl phosphoric acids was prepared by reacting 76 parts by weight of cetyl alcohol with a mixture of 17 parts of phosphorus pentoxide and 7 parts of pyrophosphoric acid at 270° F. The phosphorus pentoxide and pyrophosphoric acid were slowly added to the cetyl alcohol. The reaction was complete in two hours.

The two acids were separated by dissolving in hot alcohol (to 20% concentration) and cooling to 40° F., causing precipitation of all the di-ester. The mono-ester was extracted from the alcoholic

5

solution by means of aqueous KOH and the acid was freed by acidification with hydrochloric acid. The dicetyl phosphoric acid was recrystallized twice from 95% ethyl alcohol and once from absolute alcohol. It had a melting point of 63-64.5° C. and analyzed 5.78% phosphorus (theory 5.6%). The monocetyl phosphoric acid analyzed 9.73% phosphorus (theory 9.64%).

Both acids were white crystalline materials, the mono-ester having a flaky appearance and the di-ester, a granular appearance.

To prepare zinc monocetyl phosphate, the potassium salt was reacted with an equivalent amount of zinc chloride in alcohol solution at 150° F. over a period of 5 hours. The mixture was then cooled to precipitate white zinc monocetyl phosphate, which was washed with hot water to remove potassium chloride and unreacted zinc chloride, as shown by the appearance of only a faint cloud on treating 100 cc. of filtrate with 10 cc. of 0.05 N silver nitrate. The salt was then washed with hot ethyl alcohol and dried in a desiccator at reduced pressure.

To prepare zinc dicetyl phosphate, dicetyl phosphoric acid was reacted with zinc oxide under reflux for 7 hours, in a solvent consisting of two parts by volume of benzene and one of ethyl alcohol. The desired salt was obtained as a solid precipitate and was washed with ethyl alcohol and extracted with hot benzene. The benzene was evaporated and the precipitated salt was dried under reduced pressure. Analysis: Found, per cent Zn, 5.9; per cent P, 5.4. Theory, per cent Zn, 5.6; per cent P, 5.4.

Cadmium mono-cetyl phosphate was prepared and purified in the same manner as the corresponding zinc salt, cadmium chloride hydrate being used in place of zinc chloride. Analysis: Found per cent Cd, 29.1; per cent P, 6.6. Theory, per cent Cd, 25.9; per cent P, 7.2.

Cadmium dicetyl phosphate was prepared by reacting potassium dicetyl phosphate with an equivalent amount of cadmium chloride hydrate in alcohol at 150° F. The solid reaction product was washed with ethyl alcohol, dried, washed with hot benzene, recovered from benzene solution by evaporation of the solvent and dried under reduced pressure.

#### EXAMPLE 2

##### *Mono-tert. amylphenyl phosphoric acid and zinc and cadmium salts of the same*

p-Tert. amylphenol was reacted with an equivalent amount of phosphorus pentoxide at 300° F. for 3 hours. The reaction product was purified by recrystallization from petroleum ether to give white, flaky crystals, melting point 210-214° F. The zinc salt was prepared by refluxing one molecular proportion of the acid with 0.68 molecular proportion of zinc oxide in a solvent consisting of two parts by volume of benzene and one of ethyl alcohol for six hours. The solid reaction product was washed with 5% aqueous acetic acid to remove unreacted zinc oxide, then with ethyl alcohol to remove unreacted acid, and dried under reduced pressure.

The cadmium salt was prepared by reacting the potassium salt of mono-p-tert. amylphenyl phosphoric acid with an equivalent amount of cadmium chloride hydrate at 120° F. in ethyl alcohol. The solid reaction product which separated on cooling the mixture to room temperature was washed successively with water and ethyl alcohol to remove potassium chloride, and unreacted cadmium chloride and acid.

70

The cadmium salt was prepared by reacting the potassium salt of mono-p-tert. amylphenyl phosphoric acid with an equivalent amount of cadmium chloride hydrate at 120° F. in ethyl alcohol. The solid reaction product which separated on cooling the mixture to room temperature was washed successively with water and ethyl alcohol to remove potassium chloride, and unreacted cadmium chloride and acid.

5

Properties of the various salts of the examples are given in Table I below.

TABLE I

| Salt                                   | Melting or Decomposition Point | Appearance      | Water Solubility |
|----------------------------------------|--------------------------------|-----------------|------------------|
| Zn mono-cetyl phosphate.               | (d) 642-----                   |                 |                  |
| Cd mono-cetyl phosphate.               | (d) 585-----                   |                 |                  |
| Zn dicetyl phosphate...                | (m) 155-157...                 |                 |                  |
| Cd dicetyl phosphate...                | (d) 435-----                   |                 |                  |
| Zn mono-p-tert. amyl-phenyl phosphate. | (d) 600-612...                 | White crystals. | Practically nil. |
| Cd mono-p-tert. amyl-phenyl phosphate. | (d) 668-763...                 |                 |                  |

*d*=decomposes. *m*=melting point.

These salts were all oil-soluble, the salts of mono-esters being least oil-soluble and the salts of di-esters being most oil-soluble. In general, salts of esters containing a total of at least 20 carbon atoms are freely oil-soluble, those containing less than this being more sparingly oil-soluble.

Interatomic distances of the parent esters, and of the salts of Table I, were determined, establishing the identity of the salts. These interatomic distances, as determined by X-ray diffraction patterns, are as follows:

TABLE II  
*Interatomic distances*

| Compound | Mono-cetyl phosphoric acid | Di-cetyl phosphoric acid | Mono-p-tert. amylphenyl phosphoric acid | Zn mono-cetyl phosphate | Cd mono-cetyl phosphate | Zn dicetyl phosphate | Cd dicetyl phosphate | Zn mono-p-tert. amylphenyl phosphate | Cd mono-p-tert. amylphenyl phosphate |
|----------|----------------------------|--------------------------|-----------------------------------------|-------------------------|-------------------------|----------------------|----------------------|--------------------------------------|--------------------------------------|
|          | I II<br>4.55 30            | I II<br>11.66 10         | I II<br>9.01 25                         | I II<br>7.88 50         | I II<br>11.5 50         | I II<br>4.48 100     | I II<br>5.52 25      | I II<br>10.8 5                       | I II<br>11.0 100                     |
|          | 4.08 100                   | 5.10 50                  | 8.14 25                                 | 2.68 50                 | 8.50 20                 | 4.18 25              | 4.09 50              | 9.43 20                              | 7.38 100                             |
|          | 4.55 100                   | 5.76 50                  | 2.53 50                                 | 3.77 100                | 3.05 10                 | 7.24 20              | 5.08 25              |                                      |                                      |
|          | 4.06 25                    | 5.47 50                  | 4.93 50                                 | 1.92 10                 | 1.00 5                  | 1.77 25              | 6.58 5               | 4.44 25                              |                                      |
|          |                            |                          | 4.29 75                                 | 1.62 25                 |                         |                      | 5.99 75              | 3.56 25                              |                                      |
|          |                            |                          | 3.65 25                                 |                         |                         |                      | 5.35 25              | 3.04 50                              |                                      |
|          |                            |                          |                                         |                         |                         |                      | 4.73 25              | 2.77 25                              |                                      |
|          |                            |                          |                                         |                         |                         |                      | 4.29 25              |                                      |                                      |
|          |                            |                          |                                         |                         |                         |                      | 3.98 35              |                                      |                                      |
|          |                            |                          |                                         |                         |                         |                      | 3.86 50              |                                      |                                      |
|          |                            |                          |                                         |                         |                         |                      | 3.63 50              |                                      |                                      |
|          |                            |                          |                                         |                         |                         |                      | 3.44 20              |                                      |                                      |
|          |                            |                          |                                         |                         |                         |                      | 3.22 20              |                                      |                                      |
|          |                            |                          |                                         |                         |                         |                      | 2.94 5               |                                      |                                      |
|          |                            |                          |                                         |                         |                         |                      | 2.67 5               |                                      |                                      |
|          |                            |                          |                                         |                         |                         |                      | 2.53 5               |                                      |                                      |

Further examples of methods of preparing salts of the invention are as follows:

**EXAMPLE 3**

Zinc and cadmium dicyclohexyl phosphates

The parent acid ester is prepared by heating cyclohexanol with phosphorus pentoxide. The salts are prepared by precipitating them from an aqueous solution of the sodium or potassium salt of the parent acid, by addition of cadmium chloride or zinc acetate.

**EXAMPLE 4**

### *Zinc and cadmium naphthenyl phosphates*

These are prepared by reacting naphthyl alcohols (from reduction of naphthenic acids) with phosphorus pentoxide and precipitation of the desired salts from an aqueous solution of alkali metal salt of the parent acid ester by addition of 70 cadmium chloride or zinc acetate. 65

This application is a continuation-in-part of our copending application Serial No. 374,245, filed January 13, 1941 (now abandoned) which in turn is a continuation-in-part of application Serial No.

6

241,648, filed November 31, 1938, since issued on January 14, 1941 as United States Patent No. 2,228,659.

We claim:

- 5 1. A zinc salt of an acid ester of ortho phosphoric acid, wherein each esterifying radical is a hydrocarbon group containing not less than 5 carbon atoms.
  - 10 2. A zinc salt of an acid ester of ortho phosphoric acid, wherein each esterifying radical is a hydrocarbon group containing 5 to 20 carbon atoms, and said salt contains a total of not less than 10 carbon atoms.
  - 15 3. A zinc salt of an acid ester of ortho phosphoric acid, wherein each esterifying radical is an alkyl hydrocarbon group containing 5 to 20 carbon atoms.
  - 20 4. A zinc salt of an acid ester of ortho phosphoric acid, wherein each esterifying radical is a cycloaliphatic hydrocarbon group containing 5 to 20 carbon atoms.
  - 25 5. A zinc salt of an acid ester of ortho phosphoric acid, wherein each esterifying radical is an alkaryl hydrocarbon group containing up to 20 carbon atoms.
  - 30 6. The salts of claim 2, wherein said acid ester is a mono-ester.

TABLE II

### Interatomic distances

7. The salts of claim 2, wherein said acid ester is a di-ester.

BRUCE B. FARRINGTON.  
JAMES O. CLAYTON.  
JOHN T. RUTHERFORD.

#### REFERENCES CITED

The following references are of record in the  
60 file of this patent:

UNITED STATES PATENTS

| Number       | Name           | Date          |
|--------------|----------------|---------------|
| 1,537,572    | Zernik         | May 12, 1925  |
| 65 2,236,296 | Minik et al.   | Mar. 25, 1941 |
| 2,251,798    | Meidert et al. | Aug. 5, 1941  |
| 2,346,155    | Denison et al. | Apr. 11, 1944 |
| 2,360,302    | Etzler et al.  | Oct. 10, 1944 |
| 2,409,774    | Mack et al.    | Oct. 22, 1944 |

#### OTHER REFERENCES

Plummer et al., Jour. Chemical Soc. (London),  
pgs. 279-291 (1929).

Smith's, "Introduction to Inorganic Chemistry," 1917, 3rd Ed., pg. 763.